

SEP 23 1941

Patented July 5, 1938

2,122,856

## UNITED STATES PATENT OFFICE

2,122,856

STRAPPING MATERIAL FOR BINDING OR  
SECURING BOXES, BALES, PARCELS, AND  
OTHER PACKAGES AND PROCESS FOR  
MANUFACTURING THE SAME

Hermann Brenneisen, Paris, France

No Drawing. Application November 25, 1936,  
Serial No. 112,703. In Belgium December 4,  
1935

16 Claims. (Cl. 29—148)

The invention concerns the strapping of packing cases, bales and other parcels or packages by means of a steel strap of any cross-section (circular, flat, oval or any odd shape) and also a so-called iron strap, which is really a low grade steel strap, which is tightened around the case and then has its ends firmly joined together by any suitable means.

In practice, many different methods of joining the ends of the tightened strap are adopted. Examples are, twisting the overlapping end portions of the strap around one another, twisting one portion around the other or twisting one around itself to form a sleeve to receive the other end and then flattening down or pressing them together, forming interengaging loops on the end portions and twisting the otherwise free ends of the loops around the adjacent portions of the strap, overlapping the end portions and deforming them either with or without an engaging sleeve or sheath, according to the nature of the strapping material used.

Whatever form of the above kind of joint or knot is used, its strength, or the resistance to separation of the parts forming the joint, depends mainly, among other factors (for instance, tightness of the twist, deformation due to flattening, crimping or the like), on the coefficient of friction of the engaging surfaces of the material at the joint.

In order to obtain a joint having a high resistance to separation (all other conditions remaining unaltered), it is, therefore, important that smoothness of the engaging surfaces of the material at the joint should be avoided as much as possible, that is to say, the surfaces of the material should be provided with retaining and clinging unevennesses or prominencies.

Hitherto prominences such as teeth, projections, serrations, etc., have been formed on strapping by mechanical means, but unevennesses obtained by mechanical means are liable to weaken the strapping and are also apt to start fracture, that is to say, they may be regarded as starting points of fracture. It has also been proposed to etch a helix on one end of a wire strap so as to provide it with a rough or matt surface, the helix receiving the other smooth or untreated end and being crushed onto it.

According to the invention, the increase in the coefficient of friction is obtained by subjecting the strapping material (that is, the steel wire, band or strip), while in a heated condition, to the action of a medium which will then chemically react with the material at its surface so

as to produce the required roughness. The strapping is then cooled at any desired rate.

The heating of the strapping material should only be such as to ensure that the reaction shall occur, so as to give the desired result, and with reasonable speed, and in no case should it be such as to alter substantially the mechanical characteristics of the material as regards tensile strength or resistance to shearing. For this reason, it will generally be found necessary to heat it to at least 220° C., but in no case beyond the point of transformation or critical point of the metal.

A suitable medium for the purpose of the invention is an oxidizing medium. The heated strapping material is exposed to the oxidizing medium during the heating operation, while it is cooling or during both operations, so long as it is exposed to the oxidizing medium at a temperature not below its lowest oxidation temperature, although it may be still exposed to it even after it has cooled below this temperature, for instance, when the oxidizing medium is used also as a cooling medium.

Air is an example of a suitable oxidizing medium which may also be used as a cooling medium.

This treatment at a moderate temperature and in an oxidizing medium modifies the superficial structure of the strapping material.

It would appear from microscopic examination of steel wire strapping material treated as above in air as an oxidizing medium that the oxidation results in a coating of oxides being formed on the surface of the strapping material, which coating comprises very tenacious microscopic unevennesses or prominencies which render said surface rough or granular.

In view of the fact that the temperature of the treatment does not reach the point of transformation or critical point of the metal, it will be appreciated that there is no question of annealing or superficial hardening as these terms are generally understood in the art of steel treatment, which is borne out by tests which have shown that the mechanical characteristics of the metal (tensile strength and resistance to shearing stress) remain substantially unchanged; therefore, the result obtained is a superficial structure modification through oxidation.

It should be noted, moreover, that the external oxidation does not afterwards diffuse itself inwards in the strapping materials and that it constitutes a practical protection against rust.

Therefore, a strapping material treated in the described manner can be used after a consider-

able period following the treatment without further oxidation.

A very advantageous application of the oxidation treatment refers to wire of oval section, or 5 more generally, to wire of non-circular or any odd shaped section, obtained by the cold-rolling of hard drawn round commercial wire, sometimes termed market wire. This non-circular wire presents numerous well known advantages 10 and the alteration of the section by a cold-rolling operation is relatively easy. However, it may have the disadvantage of effecting a kind of polishing or burnishing of the surface of the wire, so that the contacting surfaces of a strapping joint made from such wire would have such 15 a low coefficient of friction, that even in the case of a very tight joint having twists of short pitch, or of wires strongly deformed, or the like, there is always the danger of the wires sliding easily relatively to one another.

If non-round wire, which has been produced by cold-rolling round wire, is submitted to the treatment according to the invention, the smooth surface of the wire due to the cold-rolling is so 25 modified that the coefficient of friction of the contact surfaces of a strapping joint made from the treated wire is considerably increased. The non-round wire so treated possesses all the advantages of a non-round strapping wire of high 30 quality with the additional guarantee of a highly resistant joint or knot.

The invention, therefore, includes as a preferred means of strapping, a non-round steel wire, obtained by the cold-rolling of a hard drawn 35 round commercial wire, and the heating of the wire, after rolling, above 220° C., but below the critical point of the metal, with a simultaneous or consecutive treatment in an oxidizing medium, the oxidizing treatment being carried out while 40 the wire is in a heated condition.

It is to be understood that the treatment according to the invention may be applied to the end portions only of the strapping material, for instance, when it is cut up into portions of definite 45 lengths.

As the treatment can be applied continuously on strapping material which travels through a heating zone, or on a strapping material in which the heat is generated by an electric current passing 50 through it, it appears to be more advantageous to apply the treatment to the whole length of the strapping material, for instance, in the case of a wire of non-round section, immediately after the cold-rolling of the round wire from 55 which it is made.

It is to be understood that the treatment according to the invention may be applied quickly, that is to say, that the strapping material need not necessarily be maintained for a long time at 60 the heating temperature, above 220° C. As soon as the required temperature has been reached, cooling can be started and thus the essential mechanical or physical characteristics of the strapping material are not substantially modified 65 or impaired.

As another example, the steel strapping material may be heated with sulphur in a non-oxidizing atmosphere at a temperature above 220° C. Iron treated in this way results in the formation 70 of iron sulphide.

The steel wire may be passed through a box having a layer of sulphur below and spaced from the wire and a gasoline flame may be directed into the box above and onto the wire. This results in a matt and rather dark and dull blue 75

surface on the wire. Tests with strapping composed of a hard steel commercial wire of oval section of a breaking strength of 195 kgs. treated in this way showed that the wire of a twisted tie broke between 160-172 kgs., but the twisted joint or tie did not unwind.

Having now described my invention what I claim as new and desire to secure by Letters Patent is:

1. Metal strapping of any shape for strapping 10 boxes, parcels, bales, packages and containers of any kind, the ends of which are adapted to be joined together, provided with a superficial adhering coat of a sulphide of the metal of which said strapping is made. 15

2. Steel strapping of any shape for strapping boxes, parcels, bales, packages and containers of any kind, the ends of which are adapted to be joined together, provided with a superficial adhering coat of iron sulphide. 20

3. Steel strapping for strapping boxes, parcels, bales, packages and containers of any kind, the ends of which are adapted to be joined together, comprising a steel wire having a non-round cross section and provided with a superficial adhering 25 coat of a stable compound of iron.

4. Steel strapping for strapping boxes, parcels, bales, packages and containers of any kind, the ends of which are adapted to be joined together, comprising a steel wire having a non-round cross 30 section and provided with a superficial adhering coat of iron oxide.

5. Steel strapping for strapping boxes, parcels, bales, packages and containers of any kind, the ends of which are adapted to be joined together, comprising a steel wire having a non-round cross 35 section and provided with a superficial adhering coat of iron sulphide.

6. Metal strapping of any shape for strapping boxes, parcels, bales, packages and containers of 40 any kind, comprising a length of strapping material, the ends of which are adapted to be joined together, one at least of said ends being provided with a superficial adhering coat of a stable compound of the metal of which said strapping is 45 made.

7. A process for manufacturing metal strapping of any shape for strapping boxes, parcels, bales, packages and containers of any kind, which consists in heating the strapping metal to a temperature above 220° C. but below the critical point of the metal, and submitting the surface of said metal while hot to the action of a medium adapted to form with said metal a stable adhering compound. 55

8. A process for manufacturing metal strapping of any shape for strapping boxes, parcels, bales, packages and containers of any kind, which consists in heating the strapping metal to a temperature above 220° C., but below the critical 60 point of the metal, and submitting the surface of said metal while hot to the action of an oxidizing medium adapted to form an oxide with said metal.

9. A process for manufacturing metal strapping of any shape for strapping boxes, parcels, bales, packages and containers of any kind, which consists in heating the strapping metal to a temperature above 220° C., but below the critical 65 point of the metal, and submitting the surface of said metal while hot to the action of sulphur adapted to form a sulphide with said metal.

10. A process according to claim 8, in which air is used as the oxidizing medium.

11. A process for manufacturing metal strapping 75

ping of any shape for strapping boxes, parcels, bales, packages and containers of any kind, which consists in exposing said metal strapping to air, passing through said metal strapping an electric current adapted to raise its temperature above 220° C. but below the critical point of the metal, whereby the surface of said metal is coated with oxide, and allowing the metal to cool.

5 12. A process for manufacturing metal strap-  
ping of any shape for strapping boxes, parcels, bales, packages and containers of any kind, which consists in heating said metal strapping in a sulphurous atmosphere, to raise its temperature above 220° C., but below the critical point of the  
10 metal, whereby the surface of said metal is coated with sulphide, and allowing the metal to cool.

15 13. A process for manufacturing metal strap-

ping for strapping boxes, parcels, bales, packages and containers of any kind, which consists in cold rolling hard drawn round steel wire into non-round wire, heating the non-round wire to a temperature above 220° C., but below the critical 5 point of the metal, and subjecting the surface of said wire while hot to the action of a medium adapted to form with said metal a stable adhering coat.

14. A process according to claim 13, in which 10 the heating of the wire is effected immediately following the cold rolling operation.

15. A process according to claim 13, in which said medium is an oxidizing medium.

16. A process according to claim 13, in which 15 said medium is a sulphurous medium.

HERMANN BRENNEISEN.